

H. T. MAITLAND,  
PROCESS OF TREATING HYDROCARBON OILS,  
APPLICATION FILED APR. 15, 1919.

1,425,883.

Patented Aug. 15, 1922.



WITNESS:

John R. Mitchell.

INVENTOR

Harold T. Maitland

BY

Frank J. Busser

ATTORNEY

# UNITED STATES PATENT OFFICE.

HAROLD T. MAITLAND, OF MARCUS HOOK, PENNSYLVANIA, ASSIGNOR TO SUN COMPANY, OF PHILADELPHIA, PENNSYLVANIA, A CORPORATION OF NEW JERSEY.

## PROCESS OF TREATING HYDROCARBON OILS.

1,425,883.

Specification of Letters Patent. Patented Aug. 15, 1922.

Application filed April 15, 1919. Serial No. 290,228.

To all whom it may concern:

Be it known that I, HAROLD T. MAITLAND, a citizen of the United States, residing at Marcus Hook, county of Delaware, and 5 State of Pennsylvania, have invented a new and useful Improvement in Processes of Treating Hydrocarbon Oils, of which the following is a full, clear, and exact description, reference being had to the accompanying 10 drawings, which form a part of this specification.

The object of my invention is to produce, by treating mineral oils, saponifiable oils or organic compounds which will have certain 15 characteristics of animal oils, vegetable oils and resins and which are adapted for various uses, some of the principal of which are for the manufacture of soaps, hydrogenated compounds, greases, drying oils, cutting oils, 20 nitrated, sulphonated and chlorinated compounds, and addition, substitution or condensation products, some of which have antiseptic and medicinal properties.

The derivative from mineral oil produced 25 by my process has a peculiar characteristic which no other known derivative from mineral oil possesses, in that it is both a water-insoluble and saponifiable product possessing, in the main, when saponified, the qualities of ordinary soaps made from oil of 30 vegetable or animal origin. The product, in the preferred forms in which I have made it, has also the following specific characteristics: It is odorless, does not become rancid, 35 and when saponified it is soluble in all proportions with water and is partially soluble in mineral oil, the degree of its solubility depending upon the character of the oil.

The production from mineral oil of sulfo-acids or sulfonic compounds which are saponifiable and when saponified exhibit some 40 of the characteristics of ordinary soap is known. These sulfonated acids, however, are quite different from my novel product 45 both in constitution and in certain essential characteristics. Thus the sulfonated acids contain, as their name implies, a large percentage of sulfur, they are soluble in water, and when saponified they do not undergo the 50 process of hydrolytic decomposition which occurs with ordinary soaps. The sulfur content of my products, on the contrary, is

scarcely more than a trace, and exists chiefly in the form of sulfates, which are there as impurities. My product, therefore, is not 55 a sulfo-acid or a sulfonic compound in any sense, as it is insoluble in water, and it behaves, when saponified, like ordinary soap in that it undergoes the same character of hydrolytic decomposition and exhibits most 60 other, and probably all other, important qualities which characterize ordinary soaps.

My new product cannot, by reason of its novelty, be too specifically designated. It is, however, undoubtedly a saponifiable oil or 65 a series of oils and it is scarcely questionable that it is an organic acid of the resin group.

The main advantage of my new product is its cheapness, by reason of the cheapness of mineral oils as compared 70 with animal and vegetable oils. It has, however, not only the economical advantage of being a derivative from mineral oils, but it has the further economical advantage 75 of being a derivative from materials which are by-products in the manufacture of lubricating oils and other standard refined products from crude oils, which by-products have hitherto either been wasted or only partially utilized for the manufacture of 80 products which command a comparatively small price. My product has a much greater commercial value than lubricating oil itself, making it profitable to so conduct the whole refining process as to make the 85 production of my new product the chief object.

In an application filed April 15, 1919, Serial No. 290,227, I have set forth two processes having certain novel features in 90 common, which I have therein claimed. I have also claimed therein, specifically, one of the two processes. The present application is confined to the disclosure of the other process, which is herein specifically 95 claimed.

In the accompanying drawing, the figure is a vertical section of a mechanical masticator and digester which I prefer to use in carrying out my process.

It will be understood, however, that the use of any particular apparatus is not essential to the execution of the process; and while the apparatus herein described

and illustrated, as well as the precise details of treatment herein set forth, have been demonstrated to be efficient by practical commercial use, it is not intended to limit 5 or restrict the invention within a narrower scope than the claims define.

While any crude petroleum is possibly or probably adapted for use in the execution of my processes, I prefer to use Texas crude 10 oil, or a crude petroleum of that nature on account of the particular group of hydrocarbons and their mobility to conversion which are found in an oil of this kind. The yield of saponifiable oils is probably increased 15 by the particular distilling process which I preferably employ to secure the so-called lubricating oil stock from which both lubricating oil and my new product are made, and I shall therefore briefly describe 20 such distilling process; although it will be understood that the essential steps of my process may be practiced starting with any lubricating oil stock or distillate, or at least any lubricating oil stock or distillate made by distilling crude petroleum of 25 the proper grade in the ordinary way.

I first take the crude petroleum and subject it to a preliminary distillation in which all of the crude product is distilled off except a relatively small percentage of 30 residuum. The distillates are then subjected to a second distillation, the heavier product remaining in the still being the stock from which lubricating oil may be made. The 35 second distillate is then redistilled, light oils being distilled off, the part remaining also being adapted for use as lubricating stock.

While some saponifiable compounds may be separated from the mineral oil by treatment 40 with fuller's earth or bone char, followed by extraction of the saponifiable compounds from the above mentioned materials with some solvent such as alcohol, ether, benzol, carbon bisulfide, etc., I prefer to 45 treat them successively with an acid and an alkali, either first treating with an acid and then with an alkali, or the reverse. A certain group of these saponifiable oils may be removed by first precipitating them with an 50 alkali and removing them before treating with sulfuric acid; or I may proceed in the usual way, namely: by first treating the lubricating stock with an acid, preferably sulfuric acid, with agitation, followed by 55 settlement. If sulfuric acid be used, it should not be the anhydride, or even fuming acid, as otherwise sulfo-acids will be formed, which may be difficult or impossible to eliminate, or which may make impossible the 60 production of the water-insoluble organic acid sought. As a specific example, 2300 barrels of lubricating stock are thoroughly agitated with approximately 75 barrels of concentrated sulfuric acid (93.5%  $H_2SO_4$ ) 65 and settlement, under appropriate tempera-

ture conditions, is allowed. The mixture of oil and acid separates into three distinct layers.

The top layer "A" consists of about 2175 barrels of treated lubricating stock, with approximately .75% sulfuric acid in suspension. The treatment of this layer, for the purpose of producing a saponifiable oil or organic acid having the characteristics hereinbefore enumerated, is set forth in said 75 application Serial No. 290,227, filed April 15, 1919, and is not herein described.

The middle layer "B" is composed of approximately 180 barrels of a mixture of sludge and sulfuric acid, the content of the 80 latter being about 30 per cent.

The lower layer "C" consists of a small amount of sulfuric acid with some sludge in solution.

The lower layer "C" should be drawn off 85 and concentrated.

Then the layer "B" (or layers "B" and "C" if the latter is not separately drawn off), to the treatment of which my process is directed, is subjected to the concurrent 90 action of water and mechanical mastication. The water should be maintained below the boiling point, although it may, if desired, exceed the boiling point toward the end of the operation. The water is preferably continuously introduced during the operation of mastication and steam is introduced with the water to maintain the water at the desired temperature.

The special mechanical masticator and digester which I prefer to employ is equipped with a steam jacket *a* built to withstand a pressure of one hundred pounds to the square inch. The inside of the digester as well as the movable parts contained within 105 it are covered with some acid resisting metal or composition: Special masticating and stirring paddles *b* with a certain sweep or pitch are arranged to revolve with a lifting and opposing effect, while stationary 110 interfering bars *c* serve the double purpose of masticating the sludge and supporting the shafts *d* and *e*. The undermost paddle *f* is hollow and operated by the hollow vertical shaft *d* which moves in an opposite 115 direction to the hollow shaft *e* containing it. The edges of this paddle which, in rotation, are at the rear, are provided with small openings *g*, through which water, air or steam, or a mixture of two or all of these, 120 may be introduced into the bottom of the digester by means of the hollow shaft *d*. The bottom of the digester is so constructed that large quantities of water, air or steam, or a mixture of them, may be introduced by 125 means of an auxiliary pipe or pipes *h*. The annular space between the two shafts is flushed with steam or water, entering at *i*, so that corrosive chemicals do not come in contact with the unprotected surfaces. Be- 130

- fore the sludge is introduced, the digester is partially filled with cold water at a temperature of approximately 20 degrees C. The desired temperature is maintained throughout the operation by means of the steam jacket and live steam blown into the contents through pipes *d* and *h*. The introduction of the washing liquid may be intermittent, but is preferably continuous, the surplus liquid passing upward through the sludge and out through an overflow *k*, carrying with it the undesirable mineral acid and certain other compounds which may be subsequently treated but the treatment of which forms no part of the present invention. The driving mechanism is so adjusted that the velocity of the masticators or paddles may be diminished or increased at will. The temperature of the contents and the velocity of the masticators are governed entirely by the condition of the sludge as the operation proceeds. The sludge is tested for mineral acidity at certain intervals and when the mineral acid content has been reduced to such an extent (say to approximately two per cent) as to give no trouble in the manufacture of the products desired from the sludge, the washing is stopped and the excess washing liquid is syphoned or drawn off. During the first part of the operation it is important that no air be permitted to be mixed with the sludge, as the buoyant air with the sulfur dioxide causes the small particles of sludge to rise to the surface and to be carried away with the washing liquid. The residual compounds settling to the bottom of digester are saponifiable oils containing some dissolved or suspended mineral oil.
- The product of this process is a water-insoluble organic acid, is practically odorless, does not become rancid, and may be readily saponified with caustic alkali or other suitable alkali. The saponified product is soluble in all proportions with water, displays the principal qualities of ordinary soap, and is partially soluble in mineral oil, the degree of its solubility depending upon the character of the oil. The soap forms with water a colloidal solution similar to that formed with water by any soap of animal or vegetable origin. Such solution, upon drying, partially hydrolyzes and does not readily dissolve in water the second time; making an ideal road oil or dust preventative. The soap, when mixed with mineral oil and water, forms a homogenous emulsion. The sulfur content of the product is about 0.4 per cent. This practically negligible proportion of sulfur probably exists as sulfuric acid or sulfates whose absolutely complete removal has not been effected.
- I do not herein claim the product produced by my process, as the same is claimed in a separate application filed April 15, 1919, Serial No. 290,229.
- Having now fully described my invention, what I claim and desire to protect by Letters Patent is:
1. The process of making a water-insoluble saponifiable oil from the sludge produced in the treatment with mineral acid of mineral oil stock, which comprises subjecting the sludge to mechanical mastication and concurrently therewith causing water to impenetrate and wash the sludge and dissolve contained mineral acid, the water being heated to such a temperature as to render the sludge of the proper consistency for working, and during the process of washing and mastication supplying fresh water and carrying off the water that has been used for washing, and continuing the process until the mineral acid content is sufficiently reduced to leave the water-insoluble saponifiable oil specified. 75
2. The process of making a water-insoluble saponifiable oil from the sludge produced in the treatment with mineral acid of mineral oil stock, which comprises subjecting a body of sludge to mechanical mastication and concurrently therewith causing a body of hot water maintained below the boiling point to flow substantially continuously into and upwardly through the body of sludge and outflow at the top, thereby impenetrating and washing the sludge with a volume of water greatly in excess of the volume of water that at any given time is acting upon the sludge, the process continuing until the mineral acid content is reduced to the point required to leave the water-insoluble saponifiable oil specified. 90
3. In the manufacture of a water-insoluble saponifiable product from mineral oil, the process which comprises distilling from the petroleum a relatively heavy distillate adapted for lubricating oil stock, treating the same with sulfuric acid and separating out the acid sludge, subjecting the sludge to mechanical mastication and concurrently therewith causing water to impenetrate and wash the sludge and dissolve contained mineral acid, the water being heated to such a temperature as to render the sludge of the proper consistency for working, and during the process of washing and mastication supplying fresh water and carrying off the water that has been used for washing, and continuing the process until the mineral acid content is sufficiently reduced to leave the water-insoluble saponifiable product specified. 105
4. In the manufacture of soap from mineral oil, the process which comprises distilling from the petroleum a relatively heavy distillate adapted for lubricating oil stock, treating the same with sulfuric acid and separating out the acid sludge, sub- 110
- 120
- 125
- 130

jecting the sludge to mechanical mastication and concurrently therewith causing water to impenetrate and wash the sludge and dissolve contained mineral acid, the 5 water being heated to such a temperature as to render the sludge of the proper consistency for working, and during the process of washing and mastication supplying fresh water and carrying off the water that

has been used for washing, continuing the 10 process until the mineral acid content is sufficiently reduced to leave a water-insoluble product, and saponifying said product to produce a soap.

In testimony of which invention, I have 15 hereunto set my hand, at Philadelphia, Pa., on this 28th day of March, 1919.

HAROLD T. MAITLAND.